

1

2,955,086

**METHOD OF PRODUCING A STABLE SODIUM PERBOR SILICATE COMPOSITION**

Harlow G. Hyatt, Williamsville, N.Y., assignor to Food Machinery and Chemical Corporation, New York, N.Y., a corporation of Delaware

No Drawing. Filed June 18, 1959, Ser. No. 821,323

2 Claims. (Cl. 252—99)

This invention pertains to a method of producing an active oxygen containing detergent composition, and to such a composition. It pertains more particularly to a method of producing a detergent composition having wetting, detergent and bleaching properties, and to such a composition.

This application is a continuation-in-part of application Serial Number 575,341, filed April 2, 1956 in the name of the present inventor, which is a continuation-in-part of Serial No. 215,853, filed March 15, 1951, both now abandoned.

Detergent compositions having wetting, detergent and bleaching properties are of particular value in various laundry operations. Detergent compositions having wetting and detergent properties are commonly composed of natural and/or synthetic soaps, surface active agents, and the like. If it be desired to impart bleaching properties to such a composition, a suitable bleaching agent, preferably of the active oxygen type, must be incorporated in the composition. Most bleaching agents of the active oxygen type, such as hydrogen peroxide itself, as well as its derivatives or addition products, such as sodium carbonate peroxide, sodium pyrophosphate peroxide, urea peroxide, sodium perborate, and other similar active oxygen compounds, when incorporated in a detergent composition, do not produce compositions of good bleaching activity because of their lack of stability in intimate mixture with the wetting and detergent components of the detergent composition.

Of the various bleaching agents of the active oxygen type, only sodium perbor silicate is fully compatible with the detergent and wetting components of detergent compositions, as its stability is not adversely affected by intimate contact with natural and/or synthetic soaps, surface active agents and the like, commonly used in the manufacture of detergent compositions for laundry purposes.

Sodium perbor silicate may be manufactured in a manner fully described in U.S. Patent No. 2,367,971. This method of manufacture is, however, not well suited for the large scale production of an active oxygen containing detergent composition having wetting detergent, and bleaching properties.

Detergent compositions having only wetting and detergent properties are commonly produced in a single step method by spray-drying a solution containing all the desired components of the finished product. Spray-drying of such a solution will directly produce a fine, granular powder suitable for packaging without any further processing. Incorporation of sodium perbor silicate, produced in accordance with U.S. Patent No. 2,367,971, into such a detergent composition, to provide bleaching properties thereto, would require grinding and blending it with the powder obtained by spray-drying a solution containing the wetting and detergent components of the finished composition. This is possible to do, as pointed out in the above mentioned patent, but represents a procedure undesirable from the viewpoint of the detergent

2

manufacturer. For this reason, sodium perbor silicate, in spite of its many excellent properties, has not found acceptance as the bleaching component in detergent compositions.

It is an object of this invention to provide a novel method of producing sodium perbor silicate by spray-drying.

It is a further object of this invention to provide a novel method of producing a detergent composition having wetting, detergent, and bleaching properties by spray-drying a homogeneous solution of all its components, and to provide compositions of sodium perbor silicate having unique properties.

I have found that sodium perbor silicate may be produced by spray-drying, if steps are taken to prevent the solution containing the starting materials; sodium hydroxide, sodium silicate, borax and hydrogen peroxide, from becoming gelatinous. Such gelatinization or solidification will invariably take place if the teaching of U.S. Patent No. 2,367,971 is followed. Gelatinization will, of course, make it impossible to process the solution by spray-drying, as the gelatinizing material would clog up and foul the delicate spraying mechanisms employed.

Gelatinization of the solution used in the manufacture of sodium perbor silicate can, however, be avoided safely, in accordance with the present invention, if provision is made to have present in that solution, sodium oxide  $\text{Na}_2\text{O}$  and silicon dioxide  $\text{SiO}_2$ , in the ratio of substantially 1:1 to 1:1.2. A solution containing, aside from borax and hydrogen peroxide, sodium silicate and sodium hydroxide, in amounts corresponding to the above mentioned  $\text{Na}_2\text{O}$  to  $\text{SiO}_2$  ratio, will not gelatinize and the solution may be spray-dried to produce a stable, yet free-flowing, fine granular powder ready for packaging, without further processing.

If in the process of my invention, sodium silicate 42° Baumé with a  $\text{Na}_2\text{O}$  to  $\text{SiO}_2$  ratio of approximately 1:2.5 is used together with the amount of  $\text{Na}_2\text{O}$  introduced by the prescribed amount of sodium hydroxide 38° Baumé, the  $\text{Na}_2\text{O}$  and  $\text{SiO}_2$  will then be present in the solution to be spray-dried in a ratio of approximately 1:1.13.

Substantial deviation from this  $\text{Na}_2\text{O}$  to  $\text{SiO}_2$  ratio will change, in an undesirable manner, the properties of the solution and the properties of the spray-dried product obtained from that solution. If the ratio is changed in the direction of higher  $\text{SiO}_2$  content, the solution will gelatinize and thus become impossible to spray-dry. For example, a solution with a  $\text{Na}_2\text{O}$  to  $\text{SiO}_2$  ratio of 1:3 will gelatinize quite rapidly. On the other hand, a solution containing substantially less  $\text{SiO}_2$  than corresponds to a  $\text{Na}_2\text{O}$  to  $\text{SiO}_2$  ratio of about 1:1.13 will remain fluid but, upon spray-drying, produces an end product of reduced stability.

I, therefore, prefer to provide for an  $\text{Na}_2\text{O}$  to  $\text{SiO}_2$  ratio substantially between 1:1 to 1:1.2.

The following example will serve to illustrate how the process of my invention may be carried out, but is not given as limitative, as variations in amount of materials employed are permitted over a wide range as hereinafter indicated.

**Example 1**

In a mixing tank constructed of material compatible with hydrogen peroxide and the alkalies used, in this case a tank made of stainless steel, were placed in the order given:

- About 20 lbs. of water
- About 45 lbs. of sodium silicate 42° Baumé ( $\text{Na}_2\text{O}:\text{SiO}_2=1:2.5$ )
- About 25 lbs. of sodium hydroxide 38° Baumé (32% NaOH)
- About 30 lbs. of borax, solid

After these materials had dissolved, about 17 lbs. of hydrogen peroxide 50% were added slowly and with stirring. The solution remained fluid and was not gelatinized. Then the solution was fed to a spray-drier and there processed in the customary manner to a free-flowing, dry powder, suitable for packaging without further processing. The finished product contained 6% active oxygen. It differed from the perbor silicate of U.S. Patent No. 2,367,971 in that the latter contained different proportions of components, and therefore had different properties. Only the chemical compositions of this invention, having the described ratio of  $\text{Na}_2\text{O}$  to  $\text{SiO}_2$ , can be spray-dried to provide the unique perbor silicate products, and the unique detergent compositions containing them, of this invention. These products and detergent compositions have a combination of stability, combined with free-flowability, not found in perbor silicates having chemical compositions outside the present range of compositions.

Certain variations in the composition of the solution to be spray-dried are possible. Thus, if it is desired to produce a product containing only 3% active oxygen, the amount of hydrogen peroxide 50% may be reduced from 17 lbs. to about 8 lbs. Also, hydrogen peroxide of other concentration may be used, such as the commercially produced solutions containing 27.5% or 35% of hydrogen peroxide by weight. The sodium hydroxide, borax and sodium silicate content of the solution may also be varied. If the percentage of these components is increased, the overall effect will be approximately the same as the effect obtained by reducing the percentage of hydrogen peroxide.

My invention also permits the production of a detergent composition having wetting, detergent and bleaching properties, by spray-drying a homogeneous solution containing not only the sodium silicate, sodium hydroxide, borax and hydrogen peroxide required to form sodium perbor silicate, but also additional surface active wetting and/or detergent agents, such as fatty acid soaps, synthetic detergents and the like. Such a procedure is illustrated by the following example.

#### Example 2

In a mixing tank constructed of material compatible with hydrogen peroxide and the alkalies used, in this case a tank made of ceramic material, were first placed about 800 lbs. of water. Such a relatively large quantity of water is required to provide enough solvent to dissolve the amount of synthetic detergent used in this example. Then were added, with stirring, and in the order given:

About 42 lbs. of sodium silicate 42° Baumé ( $\text{Na}_2\text{O}:\text{SiO}_2=1:2.5$ )

About 21 lbs. of sodium hydroxide 38° Baumé (32%  $\text{NaOH}$ )

About 31 lbs. of borax, solid

About 200 lbs. of an alkyl aryl sodium sulfonate

After these materials had dissolved, about 27 lbs. of hydrogen peroxide 27.5% was added slowly and with stirring. Then the solution was fed to a spray-drier and there processed in the customary manner to a free-flowing, dry powder, suitable for packaging without further processing. The finished product contained 2.4% active oxygen.

It is to be understood that in place of the alkyl aryl sodium sulfonate used in this example, other surface active agents having the desired wetting and detergent properties may be added. These may be, for example, ordinary fatty acid soaps, fatty alkyl sulfates, fatty monoglyceride sulfates, carboxy methyl cellulose, polyethylene oxide based non-ionic detergents, or other materials commonly used or desired to use in detergent compositions because of their special wetting or detergent properties. Moreover, these materials may be added singly or in combination.

Thus it will be seen, that my invention permits to produce, by means commonly employed in the manufacture of powdered detergent compositions, namely, by spray-drying, detergent compositions having wetting and detergent properties based on any one or any combination of commonly used components with wetting and/or detergent properties; and bleaching as well as additional detergent properties based on sodium perbor silicate as an alkaline active oxygen containing component.

Preparation of the sodium perbor silicate in a separate step and the various grinding and blending operations necessitated thereby, are thus avoided and production of the finished product ready for packaging, is achieved in one single step. It will also be understood that a solution of caustic soda and hydrogen peroxide may be obtained by dissolving sodium peroxide in water, and the employment of such a solution is contemplated as within the scope of the invention and the claims appended here-to.

#### What is claimed is:

1. Method of producing a stable, active-oxygen containing, powdered sodium perbor silicate composition, comprising spray-drying a homogeneous free-flowing aqueous solution containing, in the indicated amounts by weight, about 4-8 parts of sodium hydroxide, about 40-50 parts of sodium silicate having a degree Baumé value of 42° and an  $\text{Na}_2\text{O}:\text{SiO}_2$  ratio of about 1:2.5, about 30 parts of borax, and at least about 4 parts of hydrogen peroxide, and in which composition the total  $\text{Na}_2\text{O}:\text{SiO}_2$  ratio is about 1:1 to 1:1.2.

2. Method of producing a stable, active-oxygen-containing, powdered sodium perbor silicate composition, comprising spray-drying a homogeneous free-flowing aqueous solution containing, in the indicated amounts by weight, about 4-8 parts of sodium hydroxide, about 40-50 parts of sodium silicate having a degree Baumé value of 42° and an  $\text{Na}_2\text{O}:\text{SiO}_2$  ratio of about 1:2.5, about 30 parts of borax, and about 4-8.5 parts of hydrogen peroxide, and in which composition the total  $\text{Na}_2\text{O}:\text{SiO}_2$  ratio is about 1:1 to 1:1.2.

#### References Cited in the file of this patent

#### UNITED STATES PATENTS

|           |                  |               |
|-----------|------------------|---------------|
| 2,185,632 | Hill et al.      | Jan. 2, 1940  |
| 2,243,054 | Vail             | May 20, 1941  |
| 2,367,971 | Spiegler         | Jan. 23, 1945 |
| 2,423,451 | Holuba           | July 8, 1947  |
| 2,491,789 | Young            | Dec. 20, 1949 |
| 2,679,483 | Armstrong et al. | May 25, 1954  |
| 2,738,365 | Sylvester        | Mar. 13, 1956 |
| 2,868,615 | Bell             | Jan. 13, 1959 |